

## 1

2,998,456

SATURATED HYDROCARBON-VINYL ETHER  
REACTION PRODUCTS

George J. Benoit, Jr., San Anselmo, Calif., assignor to  
California Research Corporation, San Francisco, Calif.,  
a corporation of Delaware  
No Drawing. Filed June 12, 1958, Ser. No. 741,460  
3 Claims. (Cl. 260—614)

This invention pertains to certain particular compounds which are useful as lubricating oils; that is, compounds which have qualities necessary for a lubricating oil. The lubricants set forth herein are obtained by reacting a saturated hydrocarbon with a vinyl ether, or reacting a saturated hydrocarbon with an allyl ether.

In recent years, numerous synthetic oils have been prepared; these have become quite important in the field of lubrication. Synthetic oils can be tailor-made to suit the particular needs of a lubricant. For example, synthetic lubricants, because of their good viscosity index and low pour points are becoming of greater importance as lubricants for equipment such as gas turbine engines, etc.

As set forth in U.S. Patent 2,748,170, lubricants can be formed by reacting terminally unsaturated olefins with vinyl alkyl ethers, such as to form polymers which are suitable as lubricants. The resulting polymeric compounds, which have molecular weights from 400 to about 700, have considerable branching within the molecules. Thus, a particular disadvantage of the lubricant thus prepared is the relatively low viscosity index obtained.

Similarly, as described in U.S. Patent 2,691,646, olefinic hydrocarbons may be polymerized with vinyl ethers to form additives for lubricating oil compositions; such additives being useful for improving the viscosity characteristics of hydrocarbon lubricating oils.

It is a further object of this invention to prepare synthetic lubricating compositions useful as base oils by forming compounds having high viscosity indexes.

In accordance with this invention, it has been discovered that synthetic oils having outstanding characteristics can be prepared by reacting a vinyl ether, an allyl ether, or a mixture of such ethers, with a saturated hydrocarbon compound in the presence of a peroxide catalyst.

The products obtained according to this invention have excellent lubricating characteristics such that they are useful as lubricants for machinery, such as gas turbine engines, as base oils for greases, etc.

For simplification in describing this invention, the term "ethers" as used herein means "vinyl alkyl ethers," "di-vinyl ethers," "allyl alkyl ethers" and "diallyl ethers." The ethers may be described by the structural formula:



wherein  $R_1$  represents a vinyl or allyl radical, and  $R_2$  is a vinyl radical, an allyl radical, or an alkyl group having from 1 to 5 carbon atoms;  $R_1$  and  $R_2$  may be the same.

For purposes of this invention, it is preferred that the ethers have a total of from 3 to 6 carbon atoms.

Examples of ethers of this invention include vinyl ethyl ether, vinyl propyl ether, vinyl butyl ether, vinyl pentyl ether, vinyl hexyl ether, vinyl allyl ether, allyl ethyl ether, allyl butyl ether, allyl pentyl ether, diallyl ether, etc.

The saturated hydrocarbons with which these ethers are reacted contain from 10 to 25 carbon atoms; preferably, these saturated hydrocarbons are aliphatic hydrocarbons containing from 14 to 20 carbon atoms. These hydrocarbons are exemplified as follows: n-decane, 2-methyldecane, n-dodecane, n-tetradecane, n-hexadecane, n-octadecane, 4-methylhexadecane, n-eicosane, etc. It is preferable to use straight-chain saturated hydrocarbons, or hydrocarbons having low degree of branching. Oils

## 2

having higher V.I. are obtained by using hydrocarbons having low degree of branching.

The catalysts used herein in the preparation of these new synthetic oils include dialkyl peroxides, alkyl hydroperoxides, diacyl peroxides, and mixtures of such peroxides. Preferably, however, the peroxide employed is one of the dialkyl variety such as for example, di-(tertiary butyl) peroxide, methyl ethyl peroxide, di-(secondary butyl) peroxide, or the like. Di-(tertiary butyl) peroxide is preferred, because it has the advantage of commercial availability, and it is relatively stable.

The products formed by reacting the ether with the hydrocarbons should contain, on the average, from about 1 to 5 ether groups per hydrocarbon molecule. The choice of hydrocarbon employed is determined by the desired viscosity of the final lubricant. Increasing the number of attached ether groups beyond about 5 yield oils, the V.I.'s of which are lower than desired. Normally it is preferred to use straight-chain hydrocarbons having 14 to 20 carbon atoms per molecule reacted with vinyl or allyl ethers having 4 to 6 carbon atoms in which the reaction product has about 2 to 3 ether groups attached to the hydrocarbon.

The products useful herein as lubricants are obtained by reacting from 1 mol to 5 mols of an ether with from 5 mols to 1 mol of a saturated hydrocarbon at temperatures ranging from 120 to 200° C., using a catalyst such as di-(tertiary-butyl) peroxide.

The following examples illustrate the preparation of new synthetic oils by the reaction of saturated hydrocarbons with ethers described herein.

EXAMPLE 1.—REACTION OF VINYL ETHER  
WITH CETANE

A mixture of 500 grams of cetane and 10 grams of di-tertiary-butyl peroxide was placed in a stainless steel bomb, which was then capped and flushed with nitrogen. 40 grams of vinyl methyl ether was then pumped into the bomb, and the resulting mixture was then heated to 160° C. and maintained at about that temperature (i.e., 152° C. to 160° C.) for a period of 12 hours, then cooled to room temperature, and the liquid removed. The resulting product was fractionally distilled. After the removal of the unreacted cetane, a fraction described hereinbelow as fraction Number 1 was obtained. Physical properties and analyses of fraction No. 1 and the bottoms are set forth hereinbelow in Table 1.

Table 1

|                                   | Fraction<br>No. 1 | (Theory<br>for One<br>Vinyl<br>Ether<br>Group<br>Per Mol-<br>ecule) | Bottoms | (Theory<br>for Two<br>Vinyl<br>Ether<br>Groups/<br>Mole-<br>cule) |
|-----------------------------------|-------------------|---------------------------------------------------------------------|---------|-------------------------------------------------------------------|
| Carbon, percent.....              | 79.4              | 80.1                                                                | 77.3    | 77.1                                                              |
| Hydrogen, percent.....            | 13.9              | 14.2                                                                | 12.8    | 13.5                                                              |
| Oxygen, percent (Diff.).....      | 6.7               | 5.6                                                                 | 9.9     | 9.3                                                               |
| Molecular Weight.....             | 267               | 284.5                                                               | 297     | 342.6                                                             |
| Viscosity—<br>at 100° F., cs..... | 5.10              | .....                                                               | 28.9    | .....                                                             |
| at 210° F., cs.....               | 1.71              | .....                                                               | 5.32    | .....                                                             |
| Viscosity Index.....              | .....             | .....                                                               | 129     | .....                                                             |

Fraction No. 1 and the bottoms were both analyzed by infrared spectroscopy. The analyses showed strong ether bands at approximately 8.5 microns in fraction

No. 1 and the bottoms, and a strong band at 13.8 microns (also in fraction No. 1 and the bottoms) which indicated straight chain hydrocarbons.

EXAMPLE 2.—REACTION OF DIALLYL ETHER  
WITH CETANE

A mixture of 300 grams of cetane, 50 grams of diallyl ether and 3 grams of di-(tertiary butyl)-peroxide was

charged to a stainless steel bomb. The whole mixture was heated at 135° C. for 12 hours under a blanket of nitrogen. A liquid product was obtained and fractionated. The unreacted cetane was removed, leaving a bottoms which had the following characteristics:

| Characteristics:         | Weight percent |
|--------------------------|----------------|
| Carbon                   | 80.2           |
| Hydrogen                 | 13.0           |
| Oxygen                   | 6.8            |
| Molecular weight         | 350            |
| Viscosity at 100° F., cs | 34.0           |
| Viscosity at 210° F., cs | 6.82           |
| Viscosity index          | 153            |

The oils described herein may be base oils for lubricating compositions used for the lubrication of gas turbine engines, for grease compositions, for hydraulic fluids, etc. In addition to the base oils described herein, the lubricating compositions may contain oxidation inhibitors, lubricity agents, extreme pressure agents, oiliness agents, corrosion inhibitors, etc.

I claim:

1. A product having the characteristics of an oil of lubricating viscosity obtained by reacting from 5 to 1 mols of a straight-chain saturated hydrocarbon contain-

ing from 10 to 25 carbon atoms with from 1 to 5 mols of an ether at temperatures in the range of 120° C. and 200° C., using a di(tertiarybutyl) peroxide catalyst, said ether characterized by the formula:



wherein  $R_1$  is an unsaturated radical selected from the group consisting of vinyl and allyl radicals, and  $R_2$  is a radical selected from the group consisting of vinyl radical, allyl radical, and alkyl radicals containing from 1 to 5 carbon atoms, fractionating the reaction mixture to recover products having from 1 to 5 ether groups per molecule.

- 10 2. A product of claim 1 wherein  $R_1$  is a vinyl radical.  
15 3. The product of claim 1 where  $R_1$  is an allyl radical.

References Cited in the file of this patent

UNITED STATES PATENTS

- 20 2,391,920 Peterson ----- Jan. 1, 1946  
2,748,170 Benoit et al. ----- May 29, 1956

OTHER REFERENCES

- Schildknecht, et al.: Ind. and Eng. Chem., volume 41  
25 (1949), pages 2891-2893.